

## UNITED STATES PATENT OFFICE

2,489,384

BENZENE-AZO-BENZENE-AZO-OLEYL  
PHENOL

Henry Charles Olpin, Kenneth Ronald House, and  
John Wright, Spondon, near Derby, England,  
assignors to Celanese Corporation of America,  
a corporation of Delaware

No Drawing. Application July 9, 1946, Serial No.  
682,294. In Great Britain July 20, 1945

1 Claim. (Cl. 260—186)

1

This invention relates to the production of coloured fibres, foils, films or the like of cellulose acetate or other cellulose esters or ethers or of other fibre- or film-forming materials which are soluble in organic liquids.

U. S. Patent No. 2,420,008 and U. S. Patent No. 2,393,652 describe the spinning of coloured fibres from solutions of fibre-forming materials, the said solutions being coloured with a dye having therein a mono-valent aliphatic radicle free from sulphonic acid carboxylic groups, the said aliphatic radicle containing at least 8 carbon atoms united by carbon to carbon linkages, and particularly a mono-valent aliphatic hydrocarbon radicle containing at least 8 carbon atoms. Preferably the dyes are free from sulphonic and carboxylic groups. In this way it is possible to obtain coloured fibres which are very resistant to loss of colour when subjected to washing. Further, coloured fibres can be produced which are bright in shade and lack the undesirable greasy appearance which so often characterises fibres spun from solutions coloured with pigments. The latter feature seems to be due to the fact that the dye is largely or wholly in solution in the spinning solution and not merely suspended therein as in the case of a pigment. Solubility of the dye in the spinning solution is also of great advantage from the point of view of preparing homogeneous spinning solutions containing a definite and predetermined proportion of dye. Moreover when the dye is in solution the spinning solution is not likely to lose dye, as does a solution containing a pigment, on passage through the filters which must usually precede the spinning nozzles.

We have found that the production of coloured (particularly yellow) fibres, foils, films or the like of cellulose acetate or other cellulose esters or ethers, or other fibre- or film-forming materials soluble in organic liquids can very advantageously be effected with the aid of azo dyes obtainable by coupling diazo compounds with phenols having as nuclear substituents aliphatic radicles containing at least 8 carbon atoms, but preferably at least 12 carbon atoms, united by carbon to carbon linkages. The aliphatic radicles should be free from sulphonic and carboxylic groups. These dyes can be regarded as hydroxy aryl-azo-aryl compounds having the aliphatic

2

phatic radicle in question as a substituent in the aryl nucleus carrying the hydroxyl group. We have found that dyes of this type are as a class yellow and have very good solubility in organic liquids, notably acetone, so greatly facilitating the preparation of coloured spinning solutions. Moreover cellulose acetate and other fibres coloured with the dyes are very resistant to removal of the dye by washing and like hot aqueous treatments.

The aliphatic radicles are preferably hydrocarbon radicles and may be saturated or unsaturated and may comprise either a straight chain of carbon atoms or a branched chain of carbon atoms. Again the aliphatic radicles may be either primary, secondary, or tertiary, that is the carbon atom thereof at which the radicle is attached to the phenol nucleus may be directly attached to one, two, or three other carbon atoms of the aliphatic radicle. It is advantageous that the aliphatic radicle should contain a chain of at least 6 or 8 carbon atoms counting from and including the carbon atom at which the radicle is attached to the phenol nucleus. In general the presence of an unsaturated radicle such as the oleyl radicle  $C_{18}H_{35}$ —leads to a dye which is considerably more soluble in acetone than is the dye containing the corresponding saturated aliphatic radicle.

As examples of phenols which may be used in the preparation of the dyes may be mentioned the alkyl phenols obtainable by heating a phenol, for example phenol itself or a cresol, e. g. m-cresol, or a hydroxydiphenyl with an aliphatic alcohol containing at least 9 carbon atoms in the presence of zinc chloride. In these particular phenols the aliphatic radicle is situated in para position to the OH group if the para position of the parent phenol is free. Otherwise it is in ortho position to the OH group. The aliphatic alcohol can be for instance dodecyl alcohol, hexadecyl alcohol, octadecyl alcohol or oleyl alcohol or mixtures of two or more of these alcohols. By oleyl alcohol is meant the alcohol corresponding with oleic acid and differing therefrom in having a  $CH_2OH$  group in place of the  $COOH$  group. The alkyl phenols obtainable by heating phenols with oleyl alcohol in the presence of zinc chloride are hereinafter referred to as oleyl phenols, and the unsaturated hydrocarbon radicle so introduced

into the phenol molecule is referred to as the oleyl radicle. Another class of phenols which may be employed are the nuclear acidyl phenols in which the acidyl radicle is that of an aliphatic carboxylic acid containing a substantial number of carbon atoms, for example at least 9, e. g. lauric acid, palmitic acid, or stearic acid. p-Lauroyl phenol is an example of such a phenol.

The diazo compounds used for the production of the dyes can be those of aniline, chloranilines, toluidines, xylidines, anisidines, or p-acidylamino anilines; e. g. p-acetylamino-aniline or p-benzoyl-amino-aniline. Again an arylamide or other amide of p-amino-benzoic acid can be used, e. g. the anilide of p-amino-benzoic acid. Further diazo compounds of amino-azo compounds can be used, for example those of amino-azo-benzene and its substitution products, e. g. amino-azo-toluene.

The dyes are preferably free from sulphonic, carboxylic and nitro groups.

As specific examples of the dyes may be mentioned those obtainable by coupling diazotised p-acetylamino-aniline, p-benzoyl-amino-aniline, or amino-azo-benzene with the dodecyl phenol obtainable by heating phenol with normal or secondary dodecyl alcohol in presence of zinc chloride or the cetyl phenol obtainable by heating phenol with cetyl alcohol in the presence of zinc chloride, or the cetyl p-hydroxydiphenyl obtainable by heating p-hydroxydiphenyl with cetyl alcohol in presence of zinc chloride or the oleylphenol obtainable by heating phenol with oleyl alcohol in presence of zinc chloride. All these dyes are yellow in shade.

Our invention includes the dyes and processes for their manufacture, as well as fibres, foils, films, or the like coloured therewith.

The proportions in which the dyes are employed in the production of coloured fibres, foils, films or the like can be within wide limits, for example from 0.5 to 2.5 per cent based on the weight of the cellulose acetate or other fibre- or film-forming material. Owing to the very high solubility in acetone cellulose acetate or other fibres or products containing very high proportions of the dyes can be produced via acetone solutions of the cellulose acetate or other materials in which the whole of the requisite dye is in solution rather than in suspension.

Either wet or dry methods may be used for spinning into fibres the solutions of the fibre-forming materials containing the dyes; thus fibres may be produced by spinning the solutions either into suitable evaporative atmospheres or into suitable coagulation baths. The invention is of special value in connection with the production of coloured cellulose acetate fibres by the spinning of acetone solutions of cellulose acetate.

The fibres may of course be assembled into yarns at the time of spinning as is commonly practised. Again the fibres may be cut into staple fibre and this, either alone or mixed with other textile fibres, e. g. wool, silk, cotton, or regenerated cellulose fibres, converted into yarn by the methods commonly employed for converting cotton or wool into yarns. Yarns consisting of or containing the coloured fibres of the invention can be formed into fabrics by weaving or knitting.

The coloured materials produced in accordance with the invention may subsequently be topped with other dyes and particularly with direct dyeing dyes for cellulose esters or ethers, for example the water-insoluble dyestuffs of the nitro diaryl-amine, azo, or amino-anthraquinone series, such

as are extensively employed for the colouration of cellulose acetate materials. The topping colouring matter may be applied either uniformly or locally according to the effects it is desired to produce. The topping colours may be applied, for instance, in aqueous solution or dispersion according to their nature, or in solution in organic solvents. A single coloured material produced in accordance with the invention can thus be utilised to yield a range of materials of different shades.

The dyes of the present invention, like those of U. S. Patent No. 2,420,008, and U. S. Patent No. 2,393,652, have as a class little or no affinity for fibres of cellulose esters or ethers or other fibre-forming materials when applied thereto in the ordinary way as aqueous dispersions. It has been found, however, that valuable colourations can be obtained by applying the dyes in the form of solutions in organic liquid media. The organic liquid media can be those referred to in U. S. Patent No. 2,384,001 in connection with the employment of arylamino-anthraquinones for colouring cellulose ester or ether materials. Again the dye liquids can be applied to the materials in any of the ways described in U. S. Patent No. 2,384,001.

The invention is of especial value in the production of coloured cellulose acetate fibre, foils, films, and the like. Similar coloured products of other fibre-forming materials soluble in organic liquids, particularly other cellulose esters or ethers, can be obtained likewise, for example of cellulose propionate, butyrate, aceto-propionate, aceto-butyrate, nitroacetate, and of methyl ethyl and benzyl celluloses, and fibres and other products of polymerised vinyl compounds.

The invention is illustrated by the following examples, the parts referred to being parts by weight:

#### Example I

100 parts of oleyl alcohol, 100 parts of phenol, and 100 parts of zinc chloride are refluxed together for 16 hours. The product is washed with 500 parts of 10% hydrochloric acid, then with water, then with caustic soda solution, and again with water.

10 parts of amino-azo-benzene is stirred into 90 parts of methylated spirit. 17 parts of hydrochloric acid of 32% strength, 100 parts of ice and 25 parts of 2N-sodium nitrite solution are then added. The diazo solution so prepared is then filtered into a solution of 17 parts of the oleyl phenol (prepared as above) in 500 parts of water containing 10 parts of concentrated ammonia, 20 parts of pyridine and 10 parts of triethanolamine. The dye is thus obtained as an oil which is very soluble in acetone. It can be termed benzene-azo-benzene-azo-oleyl phenol.

Cellulose filaments are then dry-spun from a 25% solution of cellulose acetate in acetone containing 1.5% of the dye based on the weight of the cellulose acetate. Golden yellow filaments which are non-phototropic and are of good fastness to scouring are obtained.

#### Example II

10.6 parts of p-benzoylamino-aniline (mono-benzoyl-p-phenylene diamine) are dissolved in 90 parts of hot methylated spirit, 25 parts of 2N sodium nitrite added and the whole poured into a mixture of 100 parts of ice and 17 parts of hydrochloric acid of 32% strength. After stirring for one hour the diazo solution is slowly added to 34.5 parts of oleyl phenol (prepared as described in

Example I) in 180 parts of methylated spirit and 100 parts of ice while adding ammonia to neutralise acidity. The dye separates out and after standing for two hours is separated from the water-methylated spirit mixture, washed, and dried. It is very soluble in acetone and it can be termed p-benzoylamino-benzene-azo-oleyl phenol.

Cellulose acetate filaments are then dry spun from a 25% acetone solution of cellulose acetate containing 1.5% of the dye based on the weight of the cellulose acetate. Filaments are obtained which are of a golden yellow shade very resistant to hot soaping treatments.

*Example III*

30 parts of secondary dodecyl alcohol are heated with 38 parts of phenol and 38 parts of anhydrous zinc chloride for 16 hours. After washing well with dilute hydrochloric acid and water the resulting p-sec.-dodecyl phenol is separated from residual phenol by vacuum distillation, the phenol distilling first.

The sec.-dodecyl phenol is then coupled with an equi-molecular proportion of diazotised amino-azobenzene in dilute methylated spirit and in presence of sodium carbonate. The product is extremely soluble in acetone. By spinning an acetone solution of cellulose acetate containing 1.5% of the dye on the weight of the cellulose acetate, golden yellow fibres of very good fastness to soap scouring are obtained.

The p-sec.-dodecyl phenol can similarly be coupled with diazotised p-amino-acetanilide and p-amino-benzanilide.

Having described our invention, what we desire to secure by Letters Patent is:

Benzene-azo-benzene-azo-oleyl phenol.  
HENRY CHARLES OLPIN.  
KENNETH RONALD HOUSE.  
JOHN WRIGHT.

REFERENCES CITED

The following references are of record in the file of this patent:

UNITED STATES PATENTS

|    | Number    | Name           | Date          |
|----|-----------|----------------|---------------|
| 15 | 902,021   | Sulzberger     | Oct. 27, 1908 |
|    | 2,034,668 | Reindel et al. | Mar. 17, 1936 |
|    | 2,072,252 | Ellis          | Mar. 2, 1937  |
|    | 2,083,308 | Senn           | June 8, 1937  |
|    | 2,126,841 | Thurm          | Aug. 16, 1938 |
| 20 | 2,127,478 | Crosley et al. | Aug. 16, 1938 |
|    | 2,158,283 | Haddock et al. | May 16, 1939  |
|    | 2,196,985 | Flett          | Apr. 16, 1940 |
|    | 2,266,413 | Crossley       | Dec. 16, 1941 |
|    | 2,286,317 | Stanley        | June 16, 1942 |
| 25 | 2,302,530 | Crossley       | Nov. 17, 1942 |
|    | 2,315,232 | Thurm et al.   | Mar. 30, 1943 |
|    | 2,393,652 | Olpin et al.   | Jan. 29, 1946 |
|    | 2,402,538 | Dreyfus        | June 25, 1946 |

FOREIGN PATENTS

|    | Number  | Country       | Date          |
|----|---------|---------------|---------------|
| 30 | 791,902 | France        | Oct. 7, 1935  |
|    | 558,330 | Great Britain | Dec. 31, 1943 |